

A. CHURCHWARD.  
ELECTRICAL CONNECTION.  
APPLICATION FILED JUNE 19, 1920.

1,403,231.

Patented Jan. 10, 1922.



Fig. 1.



Fig. 2.

Alexander Churchward  
Inventor  
By his Attorneys  
Williams & Pitchard

# UNITED STATES PATENT OFFICE.

ALEXANDER CHURCHWARD, OF NEW YORK, N. Y., ASSIGNOR TO WILSON WELDER & METALS CO., INC., OF BROOKLYN, NEW YORK, A CORPORATION OF NEW YORK.

## ELECTRICAL CONNECTION.

1,403,231.

Specification of Letters Patent. Patented Jan. 10, 1922.

Application filed June 19, 1920. Serial No. 390,238.

To all whom it may concern:

Be it known that I, ALEXANDER CHURCHWARD, a citizen of the United States, residing in the borough of Manhattan, city, county, and State of New York, have invented certain new and useful Improvements in Electrical Connections, of which the following is a specification.

This invention relates to improvements in means for joining electrical conductors and more particularly to means for coupling a high resistance rheostat unit to a low resistance conducting wire leading to an electrical circuit.

One object of this invention is to produce an electrical juncture connecting two terminals of widely dissimilar resistances which will have a low contact resistance and in which substantially all of the heat generated by the rheostat will be liberated in the rheostat elements and the heat generated at the juncture itself will be reduced to the minimum so that the terminals will remain comparatively cool. This construction prevents premature deterioration of the terminals and hence increases the efficiency, economy and durability of the rheostat.

Another object is to construct an electrical connection between terminals of widely variant conductances by coating the terminal having the higher resistance with a metal of a lower resistance preferably similar to that of the low resistance terminal so that the contacting metals at the joint will be similar and of substantially the same resistance. It has been discovered that with such a joint the heating effect which occurs at the juncture of two dissimilar metals is practically avoided. The utilization of this phenomenon

in practice results in immense saving of power and material. This is specially true when applied to joints which are adapted to work loose. In fact it has been discovered that even with a joint loose enough to be completely burned out at a red heat in the old form of construction, applicant's joint will remain cool and will not deteriorate.

These and other objects of my invention are set forth in the following description and claims, and illustrated in the accompanying drawings in which:

Figure 1 is a view partly in section, illustrating one embodiment of my improved electrical connection shown in its operating position on a panel.

Figure 2 is a perspective view showing the improved connection disconnected from the remainder of the rheostat.

Referring to the drawing, the numeral 10 represents a welding panel or board preferably of transite or other similar insulating material.

The welding panel 10 is provided with a circular opening 11 through which passes the round-headed bolt 12 preferably of brass. 65 Connected to the end of said bolt 12 adjacent the bolt head 12<sup>a</sup> is the terminal 13 of the rheostat unit, and at the other end is the conductor or lead 14 of copper, or the like, the latter being preferably covered with the asbestos coating 15.

The rheostat unit 13 comprises a strip of high resistance metal such as nichrome provided with flanges 16 upon its side edges and with the flattened end portion 17. The 75 end of the terminal 13 is provided with a central perforation fitting about the bolt 12 and has on both of its faces a coating of copper 17<sup>a</sup> preferably deposited by electroplating.

The deposit of metal upon the terminal of the nichrome strip should be confined to the flattened portion 17 at the extreme end so that the coating will not in any way interfere with the resistance of the rheostat unit. 85

The washers 18 and 19 also preferably of brass are arranged on the bolt 12 in contact with the opposite faces of the flattened end 17 of the rheostat terminal 13, and are held tightly in contact therewith by means 90 of the brass nut 20 threaded upon said bolt, and bearing upon the steel lock washer 21.

Located upon the other side of the nut 20 are the brass spacing washer 22 and the insulating tube 23 preferably of porcelain 95 bearing upon the welding panel 10. Upon the other side of the panel 10, the lead 14 is connected to the brass bolt 12 by means of the brass washers 24, 25 and 26, the brass nuts 27 and 28, and the lock washer 29, said 100 washers and nuts being alike in all respects to the similar parts located on the other side of the panel.

The bolthead 12<sup>a</sup> is provided with a slot 31 for the purpose of allowing ready adjustment of the pressure upon the contacting surfaces of the terminals by means of a screw-driver.

In operation the coating deposited upon the opposite surfaces of the flattened termi- 110

nal of the high resistance element will result in reducing the heat generated at the terminal to the minimum, for any given pressure existing between the contacting surfaces.

- 5 It will therefore be obvious that according to the present invention a slight loosening at the joint of the rheostat terminal is less serious than was formerly the case. Hence a rheostat is more nearly "fool proof" and 10 can be operated with a cheaper grade of labor with practically no danger of burning out of the rheostat elements which would formerly have occurred when the binding screws came loose.
- 15 The metal coating 17<sup>a</sup> may be applied to the nichrome strip otherwise than by electrodeposition, as by welding or hot rolling under pressure. In any case however, the metal of the coating must enter the pores 20 and interstices of the nichrome strip and be practically completely integrated therewith. There is thus no possibility of any air-gaps existing between the nichrome and its coating and hence the heat generated at this 25 surface is reduced to the minimum.

It has been found from actual tests with a copper plated nichrome strip that the contact resistance of the joint was reduced in some instances by more than four times. In 30 other words, the contact resistance from brass to copper plated nichrome was one-quarter of the contact resistance from brass to nichrome without any coating. Hence, the heat which is developed at the brass- 35 copper plated nichrome joint is one-quarter of the heat generated between the brass-uncoated nichrome joint.

Another important advantage of the present construction of high resistance terminal 40 is the reduction of oxidation and scale formation at the contact surfaces.

In carrying out my invention I do not desire to be limited to the precise embodiment disclosed herein, but desire it to be 45 understood that many variations may be made within the general scope of the invention.

I claim:

1. An electrical connection comprising 50 conductors in electrical contact with one another, one of said conductors consisting of an element of high electrical resistance having a metal coating of an element of lower electrical resistance and the other of said 55 conductors consisting of an element of low electrical resistance.

2. An electrical connection comprising two conducting elements in electrical contact with one another, one of said elements 60 consisting of a metal of low conductivity having a coating of a metal of higher conductivity and the other of said conductors consisting of a metal of high conductivity.

3. An electrical connection for conductors 65 comprising conductors in electrical contact

with one another, one of said conductors consisting of a metal of high electrical resistance having an electro-plated coating of a metal of lower electrical resistance and the other of said conductors consisting of a 70 metal of low electrical resistance.

4. An electrical connection of the class described comprising electrical conductors in contact with one another, one of said conductors composed of nichrome, and being 75 coated with copper, and the other of said conductors composed of brass.

5. An electrical connection of the class described comprising electrical conductors in contact with one another, one of said conductors composed of nichrome ribbon electro-plated with copper and the other of said conductors composed of brass. 80

6. An electrical connection comprising conductors in electrical contact with one another, one of said conductors consisting of an element of high electrical resistance having a coating of an element of lower electrical resistance, the other of said conductors consisting of an element of low electrical 90 resistance, and means to retain said conductors in close contact with one another under pressure. 85

7. An electrical connection comprising two conductors in electrical contact with one another, one of said conductors consisting of an element of high electrical resistance having a coating of an element of lower electrical resistance and the other of said conductors consisting of an element of low electrical 100 resistance, and means to adjustably retain said conductors in close contact with one another, under pressure. 95

8. An electrical connection comprising two elements of conducting material in electrical contact with one another, one of said elements consisting of material of high electrical resistance having its terminal coated with an element of lower electrical resistance and the other of said elements consisting of 110 an element of low electrical resistance, said element of high resistance being in the shape of a ribbon. 105

9. In an electrical connection of the class described, a nichrome ribbon resistance element having its terminal perforated and coated with a material of low resistance, a binding screw extending through the perforations in said terminal, washers on said binding screw in contact with the opposite 120 sides of the end of the terminal of said ribbon and means upon said binding screw to hold said washers in close contact with the surfaces of said ribbon. 115

10. A resistance element for a rheostat 125 comprising a flat ribbon of nichrome alloy, said ribbon having its terminal perforated and coated with copper, a brass binding screw extending through said perforation, brass washers in contact with the copper 130

- coated surface of said nichrome ribbon, said binding screw extending through an insulating panel, means for holding said washers in close contact with said ribbon, and a lead 5 connected to the opposite end of said binding screw.
11. A resistance element having its terminal coated with a metal of lower resistance.
12. A resistance element of low conductivity having its terminal coated with a material 10 of high conductivity.
13. An electrical connection comprising two dissimilar conductors clamped together, the conductor of higher specific resistance 15 being provided with a coating of a material having high electrical conductivity, said coating being molecularly integral therewith to lessen the resistance of the connection.
14. In an electrical connection, the combination with an electrical conductor, of a second conductor of dissimilar material from the first conductor adapted to be held in clamping engagement with said first conductor, the first mentioned conductor being 20 of less conductivity and provided with an
- integral surface portion of better conductivity than said first conductor and extending over the contact surface thereof.
15. In an electrical connection, the combination with an electrical conductor, of a second conductor having a lower specific resistance than the first conductor, and means for clamping said conductors in contact, the first conductor having a coating of better conductivity made integral therewith by its 30 entrance into the pores or interstices of the first mentioned conductor, said coating extending over the contact surface of its conductor.
16. In an electrical connection, a nichrome 40 conductor and a metal of higher conductivity adapted to contact therewith, the nichrome conductor having an integral copper coating extending over the surface of the nichrome which is adapted to contact with 45 the metal of higher conductivity.

In testimony whereof, I have affixed my signature to this specification.

ALEXANDER CHURCHWARD.